

## UNITED STATES PATENT OFFICE

2,308,355

## LUBRICANT FOR TEXTILES AND THE LIKE

Ivor M. Colbeth, Maplewood, N. J., assignor to  
The Baker Castor Oil Company, Jersey City,  
N. J., a corporation of New Jersey

No Drawing. Original application July 17, 1940,  
Serial No. 346,024. Divided and this application  
February 4, 1941, Serial No. 377,401

5 Claims. (Cl. 252—8.6)

This invention relates to the production of 11-12 or 12-13 oleic glycerides, or a mixture of them. The resulting product possesses a high degree of purity. It is particularly useful as a softening agent or lubricant for textile products, although its use is not limited to this particular purpose. Reference is made to my Patent 2,225,552, where a procedure is described by which a rather heterogeneous mixture of products is produced. By the present invention a synthetic glyceride is produced which is almost chemically pure and is particularly useful as a lubricant for textiles and the like. This is a division of my application Serial No. 346,024, filed July 17, 1940.

Heretofore objections and difficulties have been encountered when different sorts of oils have been used as lubricants for textiles. Among the objections that have arisen have been the development of rancidity in the oils or discoloration of the textiles by the oil or both. Some of the oils that have been used for this purpose are difficult to remove, some are quite expensive and some do not possess the desired lubricating properties.

Olive oil has heretofore proven to be one of the most satisfactory oils for lubricating textiles as it possesses great lubricating power which enables the fibers that are lubricated with it to slide over each other quite easily, and at the same time its viscosity, specific gravity and iodine value are such as to make it suitable for this purpose.

However, olive oil is not entirely satisfactory as a textile lubricant. Some of the objections to it are: it is not colorless as it contains iron and chlorophyl so that there is a tendency to stain the fabric, especially white fabrics; it possesses a noticeable odor that is not pleasing to everyone so that the use is objectionable where the odor is offensive; and the source of supply of olive oil is largely in foreign countries and the price thereof varies considerably from time to time.

Castor oil has also been used as a lubricant for textiles but is not entirely satisfactory for this purpose because it will become rancid due to oxidation that forms by-products such as peroxides.

By the present invention a lubricating oil for textiles is economically produced which possesses the desirable lubricating qualities of olive oil without its objectionable properties and is free or substantially free from the presence of impurities that would injure or discolor fabrics or interfere with the lubricating properties of the oil. The lubricating oil for textiles produced by this invention has about the same viscosity, specific gravity and iodine value as olive oil, and at the same time it does not become

rancid, it is light in color or practically water white and does not become yellow with age so that it will not stain fabrics, it is free from ingredients that form crystals or hard particles at lowered temperatures, it does not become oxidized at temperatures considerably above room temperature even in the presence of moisture, and it can be cheaply manufactured.

The lubricating oil for textiles produced by the present invention is liquid at approximately 26° C. It gradually solidifies below this temperature into a soft lard-like mass. The specific gravity and iodine value are approximately those of olive oil, and at the same time this oil does not become rancid. It is light in color or practically water white, and does not become yellow with age, so that it will not stain fabrics. It can be easily emulsified in water with borax, and, due to its non-oxidizing property, it is an excellent oil for use in the oiling of wool.

In carrying out this invention castor oil is first hydrogenated in the presence of a hydrogenating catalyst at such a temperature and pressure as to preserve intact the hydroxyl groups in the ricinoleic acid radicals of the oil. This temperature is in the neighborhood of 285° C., and palladium has been found to be one of the best catalysts to effect this sort of hydrogenation. The temperature to be used can be easily determined by making tests and examining the hydroxyl value of the products. It is to be clearly understood that no stearic acid is desired as a result of the hydrogenation, and therefore every precaution should be taken to keep the reaction conditions such as to avoid the conversion of ricinoleic acid radicals into stearic acid radicals. It has usually been found that with temperatures above 285° C. hydrogenation takes place with the formation of stearic acid radicals, and with lower temperatures very little hydrogenation takes place. Increased pressures speed up the reaction and may be as high as 15 or 20 atmospheres.

After the hydrogenation step the resulting product is freed from the catalyst by filtering. It is a wax which melts at approximately 76° to 80° C. At this stage the product is colorless when molten and is pure white in solid form.

The next step in the process consists in removing the hydroxyl group that is present on each hydroxy stearic acid radical of the glyceride. Since this hydroxy group is located on the 12th carbon atom, its removal by dehydroxylation will result in an oleic acid radical having the double bond between the 11th and 12th carbon atoms or between the 12th and 13th carbon atoms. The hydroxyl connected to the 12th carbon atom and a hydrogen atom connected to an adjacent carbon atom are removed. Since the reaction cannot be controlled to such a de-

gree of accuracy that one form of the oleic acid glyceride is produced to the exclusion of the other, there is always present a mixture of the two sorts of oleic acid radical. The proportion of these two oleic acid radicals depends to some extent upon the catalyst used and the temperature of dehydroxylation as well as the pressure.

A convenient procedure to use in dehydrating the hydroxy stearic acid radicals by removing a hydroxyl group and a hydrogen atom is to melt 10 hydrogenerated castor oil and pump it into a stainless steel tank. The temperature is then raised very rapidly in about an hour by means of electrical heaters, for example, to about 260° C. A dehydroxylating catalyst such as sulphuric acid, sodium acid sulphate, phosphoric acid, or B<sub>2</sub>O<sub>3</sub>, for example, dissolved in water so as to form a clear solution is then slowly added as a catalyst 15 to the molten material, preferably while a vacuum of from 20 mm. to 4 mm. is maintained, although maintenance of a vacuum is not absolutely necessary. The higher the vacuum the better is the color of the resulting product, and the more rapidly the reaction is brought to completion. The addition of the catalyst is continued until the iodine value of the product has reached approximately 75 to 85, or about the same as the original castor oil. The batch is then cooled to about 100° C. and filtered with the aid 20 of fuller's earth, absorbent charcoal, etc. It is desirable to effect the cooling of the finished batch in a reasonably short time, because better control of the color can be obtained thereby and polymerization and other side reactions are greatly decreased or avoided.

The product produced by this invention appears to be a nearly pure chemical compound due to the fact that dehydroxylation is effected with a compound that has only one double bond in each acid radical, so that uncertainty of what the dehydroxylated compound is is avoided as compared to the uncertainty of what the final compound is when compounds having more than one double bond are dehydroxylated.

The dehydrated hydrogenated product produced in accordance with this invention is of a light color and contains only a small amount of stearic acid, if any, but due to the higher melting point of 11-12 and 12-13 oleic acid glyceride it is liquid above 26° C. and will slowly set to a lard-like consistency at temperatures below 26° C. The mass, however, never solidifies into a hard wax-like solid, but can be easily liquefied, and may even be pumped at temperatures below 26° C. without great difficulty.

Due to the elimination of the hydroxyl in this product, oxidation products thereof do not have a strong rancid odor as it the case with castor oil. Even if this product should become oxidized, the products of oxidation are stable and free from odor due to the fact that a hydrocarbon, which is odorless, is split off instead of an aldehyde, which has an unpleasant odor. This product, therefore, makes possible the use of a castor oil product in the wool industry as it does not become rancid and is free from objectionable odors which wool would absorb.

Another one of the uses to which this product may be put is as the basic material for sulphonation to produce sulpho-oleates or sodium salts of sulphonic acids. In this condition the product dissolves very readily in water and is stable to hard water without the precipitation of calcium soaps. In general, when it is sulphonated it possesses the properties of olive oil. The product 70

may be dissolved in mineral oil as a means of improving the lubricating qualities of mineral oil. Due to its resistance to oxidation and polymerization it may then be used as a textile lubricant, as it will not cause gumming of metal parts through which yarn passes, or of any machinery on which the product is used.

Another use of this product is for the preparation of an emulsion in water. An emulsion can 10 be made by mixing the product with water and adding enough borax to form an emulsion. The proportions of this product and borax will vary, depending upon the use to which it is put. The borax causes partial saponification of the oil to 15 take place, and the subsequent emulsification of the unsaponified oil is effected by the soap that is present in the mixture. In this condition it can be used to oil wool in the usual manner without danger of spontaneous combustion occurring 20 when the yarn is dry. It can be easily removed from fabric by washing in hot water, and acts in some measure as a detergent.

About 85 percent of castor oil consists of the 25 glyceride of ricinoleic acid which has one double bond between the 9th and 10th carbon atoms and a hydroxyl group connected to the 12th carbon atom. The hydrogenation step described above 30 saturates the double bond between the 9th and 10th carbon atoms, and, when the hydrogenation is properly carried out, very little if any of the hydroxy groups are removed. The subsequent 35 dehydroxylation step removes the hydroxy groups and an adjacent hydrogen atom attached either to the 11th or 13th carbon atom in the chain. This enables a glyceride of rather uniform composition to be produced. Usually there is not 40 more than about 15 to 17 percent of stearic acid formed which is not an excessive amount. Whenever the presence of stearic acid is objectionable it can be removed by cold filtration and fractional crystallization.

What is claimed is:

1. A lubricant for textiles and the like, comprising a synthetic oleic glyceride substantially 45 free from hydroxyl groups and having substantially all double bonds connected to the 12th carbon atoms in the oleic radicals.

2. A lubricant for textiles and the like, comprising a synthetic oleic glyceride substantially 50 free from hydroxyl groups and having substantially all double bonds connected to the 12th carbon atoms in the oleic radicals, said lubricant having a melting point of about 26° C.

3. A lubricant for textiles and the like, comprising a synthetic oleic glyceride substantially 55 free from hydroxyl groups and having substantially all double bonds connected to the 12th carbon atoms in the oleic radicals, said lubricant having a melting point of about 26° C. and gradually solidifying below this temperature into a soft lard-like mass.

4. A lubricant for textiles and the like, comprising a synthetic oleic glyceride substantially 60 free from hydroxyl groups and having substantially all double bonds connected to the 12th carbon atoms in the oleic radicals, said lubricant being soluble in mineral oil.

5. A lubricant for textiles and the like, comprising a synthetic oleic glyceride substantially 65 free from hydroxyl groups and having substantially all double bonds connected to the 12th carbon atoms in the oleic radicals, said lubricant being resistant to oxidation and polymerization.